

1

2,809,935

## EXTREME PRESSURE LUBRICANT

Paul R. Chapman, Crystal Lake, Allan A. Manteuffel, Union, and George Wolfram, Des Plaines, Ill., assignors to The Pure Oil Company, Chicago, Ill., a corporation of Ohio

No Drawing. Application December 22, 1954,  
Serial No. 477,134

20 Claims. (Cl. 252—46.7)

Our invention relates to an improved extreme pressure lubricant. More particularly, our invention relates to an extreme pressure lubricant composition having polymer-inhibiting and corrosion-inhibiting properties.

Extreme pressure lubricants have found extensive use as gear lubricating fluids, such as in the lubrication of gear transmissions of trucks and other vehicles. The lubrication of gears demands lubricants of special qualities, particularly high lubricity and high film strength. When a lubricant is compressed between two moving metallic surfaces, high film strength is necessary to prevent the escape or squeezing out of said lubricant from between said surfaces, with consequent welding. The extreme pressures to which such lubricants are subjected when compressed between the gear surfaces cause a rise in internal heat which is augmented by any friction generated by lack of point-lubricity. It has been found that petroleum lubricating oil fractions alone are unsatisfactory in that they do not have requisite high lubricity and high film strength and consequently allow scoring and welding of gears on continued use, together with oil breakdown because of heat generated due to high friction, etc. This is particularly true with more or less highly refined petroleum oil fractions which tend to have lower lubricity than less highly refined fractions.

Many types of additives have been prepared and added to extreme pressure lubricant formulations for the purpose of augmenting film strength, lubricity and other desired characteristics. Fatty oils and fatty acid esters, for example, have been added in various amounts and combinations to hydrocarbon oil fractions, particularly for the purpose of furnishing "oiliness," that is to say, high lubricity. It has also been found that when sulfur-containing compounds are added to extreme pressure lubricants, film strength is somewhat increased, and recent formulations have combined ester additives with sulfur by sulfurizing said esters to provide both lubricity and film strength of high degree. Still more recently, it has been discovered that the use of phosphorus in combination with the sulfur-containing ester additives has further augmented desired film strength to a level of highly satisfactory performance. Thus, oils and fatty esters may have incorporated therein phosphorus and sulfur by reaction with any one of a number of phosphorus sulfide compounds, such as phosphorus sesquisulfide. The increased performance of phosphorus and sulfur-containing esters as additives for extreme pressure lubricants, when compared with sulfur-containing esters as additives for extreme pressure lubricants, may be seen in that the former are effective for transmissions operating at both low speed and high torque, and at high speed and low torque, whereas esters which have only been sulfurized and which are considered suitable extreme pressure additives exhibit in the extreme pressure lubricants satisfactory performance only under conditions of low speed and high torque.

Extreme pressure formulations incorporating fatty esters containing sulfur and phosphorus are not only satis-

2

factory for extreme pressure properties, but also exhibit high lubricity and high film strength, together with mild inhibition of corrosion stemming from a reduced tendency for the petroleum base oil to break down. Consequently, 5 sludge, acidic corrosive bodies, and gum-forming compounds are present in smaller amounts. However, it has been found that the normally slow rate of polymerization of some fatty esters is accelerated and promoted by the presence of phosphorus in the formulation, particularly where phosphorus appears together with sulfur. When sulfur alone is present in the formulation, that is, where the fatty oil or ester is only sulfurized rather than sulfurized-phosphorized or phosphorylated, promotion and acceleration of the fatty ester polymerization are 10 absent. The polymerization reaction has the deleterious effect on the extreme pressure lubricant formulation of producing insoluble materials which tend to clog the moving parts being lubricated, increase internal and external friction, and thereby contribute to the instability of the petroleum base oil with consequently increased production of acidic bodies and other deterioration compounds. Furthermore, the increased lubricity and film strength supplied by the extreme pressure additive are 15 dissipated by the conversion of the additive into a polymerized compound. It therefore is extremely advantageous to eliminate or greatly inhibit the polymerization reaction in the extreme pressure lubricant during storage and also during various conditions of use, that is, under increased pressure and/or increased temperature.

30 It therefore is an object of this invention to provide for inhibition of polymerization in a fatty ester-containing extreme pressure lubricant.

It is another object of this invention to impart anti-corrosion properties to an extreme pressure lubricant of 35 the fatty ester-type which contains phosphorus and sulfur compounds.

It is a still further object of this invention to provide a stable extreme pressure lubricant exhibiting inhibition of polymerization of sulfurized-phosphorized fatty esters 40 and showing increased corrosion inhibition.

In general, our invention comprises a composition incorporating a phosphorus-containing fatty ester or a phosphorus-and-sulfur-containing fatty ester, or a mixture thereof, in combination with a polymerization-inhibiting 45 and corrosion-inhibiting agent. More particularly, our invention resides in an extreme pressure lubricating composition comprising a major amount of a mineral lubricating oil, and a minor amount of a phosphorus-containing fatty ester or a phosphorus-and-sulfur-containing fatty 50 ester together with a polymerization-inhibiting and corrosion-inhibiting amount of a nitrogen-containing, fatty acid-derived aliphatic compound, such as an aliphatic amine, an aliphatic amide or an aliphatic amine salt of a fatty acid of carbon chain length of 16 to 22 carbon atoms.

The base oil in our improved extreme pressure lubricant may comprise any petroleum lubricating oil fraction, such as a neutral or bright stock oil of any suitable viscosity. Non-limiting examples of said petroleum lubricating oil 60 fraction are 150 viscosity bright stock, 170 viscosity bright stock, 160 viscosity bright stock, 200 viscosity neutral oil and 170 viscosity neutral oil. Aromatic extracts from said petroleum lubricating oil fractions are also contemplated for use as or in the base oil, for example, phenol extract from 150 viscosity bright stock, which means the aromatic extract obtained by extracting with phenol the requisite residual lubricating oil fraction and removing the phenol from the extract phase by flash vaporization, usually under reduced pressure, followed by steam stripping. Aromatic extracts of petroleum lubricating oil fractions derived from extractions with selective solvents 65 other than phenol, such as sulfur dioxide, nitrobenzene,

chlorex, furfural, dipropionitriles, hydrogen fluoride, dimethyl ammonium diethyl carbamate, etc., are also contemplated. Also within the scope of our invention are mixtures of said extract oils, mixtures of finished lubricating oil fractions, and mixtures of said extract oils with said lubricating oil fractions.

The extreme pressure additive of our composition is derived from any fatty ester of a mono-, di-, or tri-hydroxy aliphatic alcohol, which ester is soluble in the petroleum base oil utilized in the formulation. The ester preferably is of a fatty acid of 12 carbon atoms or more, and more preferably is one of a fatty acid of 16 carbon atoms or more, for example, palmitic, arachidic, behenic, palmitoleic, petroselinic, vaccenic, linolenic, eleostearic, licanic, parinaric, tariric, gadoleic, arachidonic, cetoleic, erucic, stearic, linoleic, oleic, and other fatty acids both saturated and unsaturated, such as glyceryl trioleate, methyl oleate and dioleate of propylene glycol. Castor oil, lard oil, sperm oil, degras and other fatty oils and fatty grease may also be used. An especially preferable ester is the methyl ester of tall oil fatty acids, a commercial form of which is Metalyn manufactured by the Hercules Powder Company and having the following characteristics:

|                                               |                                   |
|-----------------------------------------------|-----------------------------------|
| Percent methyl esters of rosin acids          | 45.0 (typical).                   |
| Percent methyl esters of fatty acids          | 47.0 (typical).                   |
| Percent unsaponifiable modified AOCS          |                                   |
| Ca 6b-40                                      | 8.0 max.                          |
| Saponification No. (drastic, Hercules method) | 155/170.                          |
| Acid No. (AOCS Da 14-42)                      | 5.0 max.                          |
| Iodine No. (AOCS Cd 1-25)                     | 120/130.                          |
| Acetyl value (AOCS Cd 4-40)                   | 10.0 max.                         |
| Color (Gardner 1933)                          | 12.0 max.                         |
| Specific gravity 20°/20° C                    | .95/.975.                         |
| Flash point °C. (COC)                         | 182° min.                         |
| Freezing point °C                             | 10.0° max.                        |
| Viscosity at 100° F. SUS (ASTM D445-45T)      | 70/100.                           |
| Moisture (AOCS ca 2a-5)                       | 0.1 max.                          |
| Appearance at 20°/30° C                       | Clear and free of foreign matter. |

The alcohol radical of the fatty ester, as mentioned above, may be any mono-, di-, or trihydroxy aliphatic alcohol radical, but it is preferable that the alcohol be a lower molecular weight and lower carbon chain length aliphatic alcohol, such as methyl alcohol, ethyl alcohol, n-propyl alcohol, allyl alcohol, n-butyl alcohol, isoamyl alcohol, sec.-butyl alcohol, tert.-butyl alcohol, isobutyl alcohol, isopropyl alcohol, n-amyl alcohol, tert.-amyl alcohol, glycol, glycerol, propylene glycol, trimethylene glycol and the like, whether it contains one, two or three hydroxyl radicals. The fatty ester may be used alone or in combination with other fatty esters. If a mixture is used, one or more of the esters may be sulfurized and the other esters may be phosphorized or phosphorized-sulfurized, or alternatively, all the esters may be phosphorized-sulfurized or phosphorylated. An example of a mixture is Metalyn in that it comprises a mixture of methyl esters of the fatty acids of tall oil which contains a mixture of linoleic acid, oleic acid and the resin acids, principally abietic acid. The proportions of the constituents fluctuate to some extent from sample to sample.

The fatty esters may be sulfurized by any one of a number of known methods, including the following: Elemental sulfur in the form of finely powdered sulfur may be sifted in small increments into a kettle containing the fatty ester or fatty ester mixture, for example, Metalyn. The constituents in the kettle are heated to about 270° F. to 285° F. while being vigorously agitated by a mechanical agitator. In the case of Metalyn it is preferable to react 93 parts of Metalyn with 7 parts by weight of sulfur. The ratio of Metalyn to sulfur may suitably vary from about 85 parts Metalyn with 15 parts

7  
sulfur to about 97 parts Metalyn with 3 parts sulfur. Suitable ratios are known for other fatty ester mixtures. After the addition of the sulfur to the fatty ester, the temperature of the mixture is raised to about 350° F. and the reaction is allowed to proceed for about 7-8 hours until fully completed, as indicated by a suitable test, such as a copper strip test. Shorter reaction periods may be employed where more highly active catalysts are available and fatty esters and sulfur react more quickly. During the final stages of reaction, the temperature may be allowed to rise to about 375° F. to insure complete reaction. The aforesaid copper strip test consists of immersing a copper strip in a sample of the product for one minute at 300° F., and if the copper strip remains peacock, the reaction is completed. In the case of Metalyn, the final product may contain about 6.25 percent of sulfur as the preferred quantity, although sulfurized Metalyn or other fatty esters may contain various amounts, such as 3-10 percent of sulfur. Where smaller amounts of sulfur are desired, the reaction time and/or temperature may be reduced. Conversely, if larger amounts of sulfur are to be incorporated, longer reaction times and/or higher temperatures will be required to obtain the finished product. However, temperatures in excess of 400° F. should be avoided.

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005

that it is generally undesirable to treat the Metalyn or similar esters with phosphorus sulfide in that the phosphorization reaction immediately produces some polymerization and decreased production of end-product. This situation extends to the methyl esters of tall oil as well as the ethyl, propyl, butyl and amyl esters of tall oil, and particularly to the isopropyl esters, isobutyl esters and similar branch-chain esters of tall oil. The incorporation of the phosphorus in the fatty ester is therefore preferably performed with fatty esters other than those of the tall oil type; it has been shown that mono-, di-, and trioleates of glycerol exhibit no immediate polymerization upon reaction with the phosphorus sulfide and are therefore preferred fatty esters for reaction with the phosphorus sulfide. The extreme pressure additive produced as outlined above increases the temperature stability, pressure resistivity, lubricity, and film strength, and fortifies to some extent the base oil against deterioration and formation of corrosive bodies. It may be present in any effective minor amount, such as, for example, 10 percent by weight of the final composition.

The polymerization-inhibiting and corrosion-inhibiting agent of our formulation may be present in any effective minor amount, such as 0.05-10 percent by weight of the final composition, and comprises at least one member of the class of compounds characterized as basic organic nitrogen compounds derived from at least one fatty acid containing a carbon chain length of at least 16 carbon atoms. These compounds fall into three sub-classes, the fatty amides, the fatty amines and the aliphatic amine salts or soaps of fatty acids having carbon chain lengths of at least 16 carbon atoms and not more than 22 carbon atoms. The additive must be oil-soluble or be used in conjunction with a suitable assisting agent which renders said additive oil-soluble. Mixtures of the compounds of the three sub-classes are therefore contemplated as the polymerization-inhibiting and corrosion-inhibiting additive.

The fatty amines referred to and effective as the polymerization-inhibiting and corrosion-inhibiting agents in our formulations may be only amines having at least one carbon chain of 16-22 carbon atoms. The term "fatty amines" indicates, according to current terminology, the fact that the amines were derived from fatty acids of comparable carbon chain length. Such fatty amines are saturated primary amines such as, palmitylamine, stearylamine, arachidylamine, behenylamine and the like; primary mono-unsaturated amines, such as oleylamine, palmitoleylamine, petroselinylamine, vaccenylamine, gadoleylamine, cetoleylamine and erucylamine; di-unsaturated amines, such as linoleylamine; tri-unsaturated amines, such as linolenylamine, licanylamine and eleo-stearylamine; and secondary amines such as Armeen 2C and Armeen 2HT, commercial mixtures of secondary fatty amines as shown below:

| N-alkyl radical | Armeen<br>2C,<br>Percent | Armeen<br>2HT,<br>Percent |
|-----------------|--------------------------|---------------------------|
| octyl           | 8                        |                           |
| decyl           | 9                        |                           |
| dodecyl         | 47                       |                           |
| tetradecyl      | 18                       |                           |
| hexadecyl       | 8                        | 21                        |
| octadecyl       | 10                       | 71                        |

We do not wish to be limited by the foregoing examples of illustrative amines since other C<sub>16</sub>-C<sub>22</sub> aliphatic amines may be used. Each amine must be oil-soluble or soluble in an assisting agent which is miscible with oil. Thus, taricylamine with an acetylenic linkage or triple bond is contemplated, as well as parinarylamine with four double bonds, and similar compounds. Similarly, diamines, triamines and other types of the amines of the specified

carbon chain lengths may be utilized. Oil-soluble tertiary amines having at least one carbon chain of 16-22 carbon atoms are also contemplated.

Many methods may be invoked for the preparation of the desired amines. However, one suitable method involves the reaction of a fatty acid or a fatty acid mixture with ammonia for the production of an ammonium salt of a fatty acid which when heated decomposes to a fatty amide which in turn forms an aliphatic nitrile. Upon hydrogenation the nitrile is converted into the desired fatty amine. Other methods available for the production of amines are, for example, alkylation of ammonia with chlorides of suitable carbon chain length, treatment of amides with sodium hypochlorite or sodium hypobromite, and processes such as the Hofmann reaction, the Curtius reaction and the Gabriel synthesis.

Armeen-S is a commercial product manufactured by Armour & Company, Chicago, Illinois, which comprises a mixture of fatty amines, namely 10 parts by weight of hexadecylamine, 10 parts of octadecylamine, 35 parts of octadecenylamine and 45 parts of octadecylidienylamine, that is, a palmitylamine, stearylamine, oleylamine and linoleylamine. This amine mixture is suitable for use as the polymerization-inhibiting and corrosion-inhibiting agent.

Armeen-HTD is also manufactured by Armour & Company, Chicago, Illinois, and comprises a mixture of about 25 parts by weight of hexadecylamine, 70 parts by weight of octadecylamine, and 5 parts by weight of octadecenylamine. In both of the above products the proportions of amine components may vary with different samples.

Duomeen T is a third commercial preparation of Armour & Company, Chicago, Illinois, which is also suitable for use in the composition of our invention. Duomeen T is a member of the group of fatty diamines which are more particularly described as N-alkyl trimethylene diamines and have the following general formula:



In the case of Duomeen T, the alkyl group is derived from tallow acids and is composed of a mixture of  $C_{16}$  to  $C_{18}$  normal saturated hydrocarbon chains and a  $C_{18}$  mono-unsaturated chain.

The amides of our invention which may be utilized as polymerization-inhibiting and corrosion-inhibiting agents in our composition are of comparable carbon chain length and configuration to the above-mentioned amines and are, for example, the following: stearylamide, oleylamide, palmitylamide, linoleylamide, arachidylamide, behenylamide, palmitoleylamide, petroselinylamide, vaccenylamide, gadoleylamide, cetoleylamide, erucylamide, linolenylamide, licanylamide, eleostearylamide, tarirylamide, parinarylamide and the like. The amides which are suitable may be with at least one saturated or unsaturated carbon chain ranging from C<sub>16</sub> to C<sub>22</sub>. The unsaturated amides may have one or more double or triple bonds. They may also have more than one amide radical per molecule. The methods of preparation are similar to those described above for the amines; for example, reactions of ammonia with fatty acids, followed by pyrolysis, and reactions involving esters, or organic acid chloride or anhydrides, as noted above. They may also be prepared by partial hydrolysis of nitriles. Each is oil-soluble or soluble in an oil-soluble assisting agent.

Duomeen T Dicoleate is an Armour & Company, Chicago, Illinois, commercial product which is suitable for use as the corrosion and polymer formation inhibitor and which may be characterized as a substituted diamine salt of a fatty acid. Duomeen T Dicoleate is water-insoluble and is thoroughly soluble in isopropyl alcohol, benzene, tetrachloroethylene, mineral oil, naptha, ethyl acetate, lard oil and similar substances. It is obtained by

7  
direct neutralization of Duomeen T with oleic acid and has the following structure:



Duomeen T Dioleate upon high heating breaks down to form the comparable amide and water.

Duomeen T Dioleate is typical of the aliphatic amine salts of fatty acids of carbon chain lengths of 16-22 carbon atoms wherein the amine radical has 16-22 carbon atoms. Other examples are Duomeen T distearate, Duomeen T dipalmitate, stearylamine oleate and the like. Said salts have varying degrees of stability. Each salt must either be oil-soluble or soluble in an assisting agent which in turn is soluble in oil. The amine radical of the salt may have an alkyl substituent of a total number of carbon atoms which when added to the number of carbon atoms of the amine nucleus totals 16-22 carbon atoms. Thus, for example, with amine radicals having 3 nuclear carbon atoms, an alkyl substituent of 13 to 19 carbon atoms would be present, as in Duomeen T Dioleate.

"Acryloid 150" is a commercial methacrylate ester copolymer sold under this name by Rohm & Haas and has the formula



in which R is predominantly a mixture of cetyl, lauryl and octyl groups and the molecular weight of the polymer is about 10,000 to 15,000.

8  
in. swing diameter for 5 minutes, then the supernatant oil was decanted and the tubes allowed to drain for 1 hour at room temperature. Solid residue was washed with ASTM naphtha to an oil-free state and dried at 220° F., and the tube weighed to the nearest mg.; where the residue was liquid, it was restored for 60 days, then re-centrifuged and the volume of separated liquids observed to the nearest 0.05 ml. Where the separated material was solid, average increase in weight of each tube and residue over the initial weight of the clean tube was reported in terms of percent by weight of the non-petroleum material originally in the sample. Where the separated material was liquid, the volume was reported in terms of percent by volume of the non-petroleum material originally in the sample.

10 The best results from a heat stability standpoint were obtained by combining Armeen-S and Duomeen T Dioleate as shown in blends L and M of Table I. The sulfurized Metalyn-phosphorized glyceryl trioleate extreme pressure additive of the gear lubricant used in the tests reported in the tables contains three parts by weight of sulfurized Metalyn and one part phosphorized glyceryl trioleate, the preparation of both of which is described earlier in the specification.

25 A further test showed that Armeen-S and Duomeen T Dioleate prevented the formation of polymers during the CRC-L-22 Storage Stability test when used in concentrations of about 0.1 percent or more, but concentrations of about .01 percent of the aforesaid additives failed to prevent polymerization during the test period.

30 A gear oil containing of Armeen-S was subjected to a series of bench tests, namely, the ASTM turbine oil rust

TABLE I  
Storage stability characteristics of extreme pressure lubricants

| Extreme Pressure Blend                          | A     | B     | C     | D        | E        | F     | G     | H      | I     | J        | K     | L     | M    |
|-------------------------------------------------|-------|-------|-------|----------|----------|-------|-------|--------|-------|----------|-------|-------|------|
| SAE 90 Grade Extreme Pressure Lube <sup>1</sup> | 100   | 99.8  | 99.9  | 99.8     | 99.9     | 99.8  | 99.9  | 99.8   | 99.85 | 99.85    | 99.85 | 99.85 | 99.9 |
| RD 1937 <sup>2</sup>                            | 0.2   |       |       |          |          |       |       |        |       |          |       |       |      |
| Duomeen T Dioleate                              |       | .1    | 0.2   |          |          |       |       |        |       | 0.05     | 0.1   |       |      |
| Armeen S                                        |       |       |       |          | 0.1      | 0.2   |       |        |       | 0.1      | 0.05  | 0.1   | 0.05 |
| Duomeen T                                       |       |       |       |          |          |       | 0.1   | 0.2    |       |          | 0.05  | 0.1   | 0.05 |
| Storage Stability <sup>3</sup>                  |       |       |       |          |          |       |       |        |       |          |       |       |      |
| CRC L-22 (200° F.)                              | .48   | .05   | 00    | 00       | 00       | 00    | 00    | 4 Fail | 00    | 00       | 00    | .05   | 00   |
| Time in Days                                    | 6     | 13    | 30    | 30       | 30       | 30    | 30    | 30     | 30    | 30       | 30    | 30    | 30   |
| Rating                                          | H. D. | H. D. | L. P. | V. L. P. | V. L. P. | Film  | Film  | Trace  | Trace | V. L. P. | Trace | Clear |      |
| CRC L-22 (300° F.)                              |       |       |       |          |          |       |       |        |       |          |       |       |      |
| Time in Days                                    | 1     |       | H. D. | 3        | 3        | 3     | 2     | 6      |       |          |       |       |      |
| Rating                                          | H. D. |       |       | H. D.    | H. D.    | H. D. | L. P. |        |       |          |       |       |      |

<sup>1</sup> Formulation, percent by wt. composition:  
10 (3 sulfurized Metalyn) (1 phosphorized GTO).

1 dibenzyl sulfide.

56-150 viscosity bright stock.

32-170 viscosity neutral.

1-Acryloid 150.

<sup>2</sup> RD 1937 is a soya amine oleate stabilizer similar to Duomeen T Dioleate.

<sup>3</sup> Rating for storage stability test:

Clear.

Trace.

Film.

Very light peppery deposit-V. L. P.

Light peppery deposit-L. P.

Heavy deposit-H. D.

<sup>4</sup> Two phase liquid separation.

The various combinations of Armeen-S, Duomeen T and/or Duomeen T Dioleate as polymerization-inhibiting, gear-oil additives were satisfactory for the duration of the CRC-L-22 storage stability test, which test was performed in the following manner: Two centrifuge tubes (100 ml. cone-shaped ASTM designation D96) were rinsed with naphtha, cleaned with concentrated sulfuric acid saturated with sodium or potassium dichromate, rinsed with distilled water, rinsed with 95% alcohol or S-free acetone and air-dried; they were then weighed to the nearest mg. and 100 ml. of the test lubricant placed in each tube. The tubes were then placed in storage at the desired temperature in a darkened room for 30 days. On conclusion of the storage period, the tubes were centrifuged at 1500 R. P. M. in a centrifuge of 15-17

65 test, the Modified SAE machine test and the Timken test.

The turbine oil rust test was performed according to the procedure of test method ASTM designation D665-53T and may be briefly described as follows:

70 A mixture of 300 ml. of the oil under test is stirred with 30 ml. of distilled or synthetic sea water, as required, at a temperature of 140° F. with a cylindrical steel specimen completely immersed therein, usually for a period of 24 hours. The specimen is then withdrawn and examined under normal light without magnification to determine the degree of rusting. A rusted specimen is one on which any rust spot or streak is visible by visual inspection.

75 The modified SAE machine test is performed in the following manner:

The SAE machine is equipped with a temperature-controlled oil reservoir from which the test lubricant is pumped to the test pieces. The overflow from the upper oil pot returns to the reservoir. The test cups are weighed on an analytical balance before and after the test and the weight loss is used jointly with a visual evaluation of the surfaces to provide a rating on the test oil.

|                       |          |      |
|-----------------------|----------|------|
| Break-in beam load    | lbs      | 50   |
| Break-in duration     | hrs      | 0.5  |
| Test beam load        | lbs      | 110  |
| Test duration         | hrs      | 15.8 |
| Upper shaft speed     | R. P. M. | 264  |
| Shaft ratio           | 10.4/1   |      |
| Temperature (oil pot) | ° F.     | 225  |

The SAE machine used is the SAE extreme pressure lubricant testing machine (CRC designation EL-17-545) and consists essentially of a device in which 2 cylindrical test specimens are rotated in line contact with each other and in opposite directions, with provision for controlling the speed of rotation, the slipping velocity, and the rate of applying pressure at the line contact between the rotating cylinders.

The Timken CRC designation L-18-545 test is used, a brief summary of which follows: The Timken extreme pressure lubricant testing machine (CRC designation EL-18-545) is cleaned and then about 1 pint of the test lubricant is put into it, circulated through it for 2-3 minutes and discarded. Fresh test lubricant at  $125^{\circ} \pm 5^{\circ}$  F. is placed in the machine and circulated therein for 15 minutes prior to the test. The test cup (average surface finish 20-30 microinches) is placed on the mandrel, and the test block in the holder on the machine. Test cup and block are then covered with test lubricant. When the apparatus is properly aligned and the reservoir on the machine is about 50% full of lubricant, the machine is started. The mandrel revolves at 800 R. P. M., producing rubbing speed on the test cup of 400 F. P. M. The desired load is applied to the lever arm of the machine which runs 10 minutes unless scoring occurs earlier. The test is repeated with a new surface of the test block, a new cup and a heavier load if no scoring occurs. Tests are run until the weight necessary to cause scoring is found. The width of the score on the test block is measured and the load in p. s. i. at the end of the test can be calculated as follows:

$$p. s. i. = \frac{\text{beam load (lb.)} \times 10}{\text{score width (in.)} \times \text{score length (in.)}}$$

the load-carrying capacity of the test lubricant is repeated in p. s. i. at maximum load in lbs. that can be applied without causing a score.

The results of the above tests in which Armeen-S wax incorporated with sulfurized Metalyn and phosphorized glyceryl trioleate in mineral oil as a gear oil formulation appear in Table II below:

TABLE II

| E. P. Lube                            | ITB125 | 52-194 | 80/90 SAE Oil |
|---------------------------------------|--------|--------|---------------|
| Composition by weight:                |        |        |               |
| E. P. Base                            | 10     | 10     | 13            |
| (Sulfurized Metalyn)                  | (3)    | (3)    | (5)           |
| (Phosphorized GTO)                    | (1)    | (1)    | (1)           |
| Dibenzyl disulfide                    | 1      | 1      | 1             |
| Acryloid 150 <sup>1</sup>             | 1      | 1      | 1             |
| 150 Viscosity Bright Stock            | 56     | 56     | 54            |
| 170 Viscosity Neutral Lubricating Oil | 31.9   | 32     | 31            |
| Duomeen T Dioleate                    | 0.1    |        |               |
| Viscosity 210° F. SUS                 | 83.7   | 83     | 81.7          |
| Viscosity 100° F. SUS                 | 170.9  | 779    | 759           |
| Viscosity Index                       | 107    | 108    | 108           |
| ASTM Turbine Oil Rust Test            | Passed | Failed | Failed        |
| Timken Test:                          |        |        |               |
| Beam Load, lbs.                       | 65     | 59     | 51            |
| Pressure, p. s. i.                    | 39,000 | 40,000 | 38,000        |
| Modified SAE Test                     | Passed | Passed | Failed        |
| Weight Loss in mg                     | 22.2   | 25     | 32.4          |

<sup>1</sup> Acryloid 150 is a viscosity index improver which also functions as a pour point depressant and is a methacrylate polymer.

Armeen S appears to have no adverse effect on the performance of the extreme pressure lubricant; and it inhibits rust, as shown by the ASTM turbine oil rust test, as well as preventing polymer formation.

Armeen HTD was similarly evaluated by a series of bench tests to determine its qualities as a stabilizer for gear oil formulations.

The function of dibenzyl disulfide formulations in formulations appearing in tables in this specification is to provide additional, properly available sulfur to the gear oil to assure satisfactory performance of the gear oil at low temperatures and pressures. The Armeen HTD polymerization-inhibiting additive appears to have no adverse effect on the gear oil formulation; that is, the Armeen HTD imparts its polymerization-inhibiting characteristics without depreciating the extreme pressure characteristics of the formulation.

Duomeen T. Dioleate was similarly subjected to a series of bench tests to evaluate its stability in gear oil containing sulfurized Metalyn and phosphorized glyceryl trioleate. The results appear below in Table III.

TABLE III

| 25                                    | E. P. Lube | ITB126 | 52-194 | 80/90 SAE Oil |
|---------------------------------------|------------|--------|--------|---------------|
| Composition by Weight:                |            |        |        |               |
| E. P. Base                            | 10         | 10     | 13     |               |
| (Sulfurized Metalyn)                  | (3)        | (3)    | (5)    |               |
| (Phosphorized GTO)                    | (1)        | (1)    | (1)    |               |
| Dibenzyl disulfide                    | 1          | 1      | 1      |               |
| Acryloid 150                          | 1          | 1      | 1      |               |
| 150 Viscosity Bright Stock            | 56         | 56     | 54     |               |
| 170 Viscosity Neutral Lubricating Oil | 31.9       | 32     | 31     |               |
| Duomeen T Dioleate                    | 0.1        |        |        |               |
| Viscosity 210° F. SUS                 | 83.7       | 83     | 81.7   |               |
| Viscosity 100° F. SUS                 | 170.9      | 779    | 759    |               |
| Viscosity Index                       | 107        | 108    | 108    |               |
| ASTM Turbine Oil Rust Test            | Passed     | Failed | Failed |               |
| Timken Test:                          |            |        |        |               |
| Beam Load, lbs.                       | 65         | 59     | 51     |               |
| Pressure, p. s. i.                    | 39,000     | 40,000 | 38,000 |               |
| Modified SAE Test                     | Passed     | Passed | Failed |               |
| Weight Loss in mg                     | 22.2       | 25     | 32.4   |               |

Duomeen T Dioleate had no adverse effect on the extreme pressure characteristics of the gear oil formulation, as evaluated by the modified SAE test, the Timken test, and the ASTM turbine oil rust test. It was found that 0.1 percent by weight of Duomeen T Dioleate is sufficient to prevent traces of sediment accumulating during the CRC-L-22 storage stability test and inhibits corrosion by the composition. Comparable results were obtained when sulfurized methyl esters of animal fatty esters were substituted for Metalyn in the Metalyn-phosphorized glyceryl trioleate extreme pressure additive; that is, when sulfurized methyl esters of animal fatty acids were used in combination with phosphorized glyceryl trioleate and Duomeen T Dioleate, the latter in about 0.1 percent concentration, polymerization of the extreme pressure additive in the gear oil was inhibited. Marked inhibition of corrosion by the gear oil was also noted.

A further example of the polymerization-inhibiting properties of the composition of our invention appears below:

A concentrate of 30.5 percent of Duomeen T Dioleate was prepared in SAE 80/90 grade gear oil containing sulfurized Metalyn and phosphorized glyceryl trioleate and this blend was added to 6,000 gallons gear oil base stock. The addition of the Duomeen T Dioleate concentrate was made in increments of 10 and 15 gallons while mixing was carried on by recirculating the gear oil from the bottom of the storage tank to the top with the pump. It was found that Duomeen T Dioleate prevented the further polymerization of the gear oil for the test period of 90 days, although polymers which had formed before the addition of the Duomeen T Dioleate could not be reabsorbed by the addition of said Duomeen T Dioleate, and appeared on the surface of the gear oil during the storage period.

The results with the polymerization-inhibiting and corrosion-inhibiting additives of our composition are contrasted with those obtained when comparable amounts, about 0.1 percent by weight of lower molecular weight, amines were added to sulfurized Metalyne and phosphorized glyceryl trioleate in hydrocarbon oil. When tertiary-octylamines and tertiary-butylamines were each tested by the CRC-L-22 storage stability test, having been incorporated in the above-mentioned gear oil in 0.1 percent by weight concentration, the resulting gear oil exhibited continued substantial polymer deposition and at the end of the 30 day test period the samples of the lubricant showed separation of liquid into two or more phases. In addition, the beneficial corrosion-inhibiting characteristics noted upon the addition of the polymerization-inhibiting additive of our composition were absent when the gear oil formulations containing amines with fewer than 16 carbon atoms were tested by means of the NRL static water drop test as set forth in MIL-P-17272 (ships) 18 July 1952. A summary of the test is as follows: The test specimen (1/2 inch cold-rolled steel (SAE 1020) in the form of an equilateral triangle) is polished on its dimpled side with sandpaper and placed into pure benzene, swabbed with clean gauze, placed into more pure benzene and boiled 3-4 minutes, put into petroleum ether and boiled 1 minute. The test specimen is immersed with the concave side of its dimple uppermost in a beaker containing oil so that the latter covers it to about 0.25 inch depth. The beaker containing the oil and sample is heated to  $140^{\circ} \pm 2^{\circ}$  F. for 1 hour and removed. A drop of water, 0.2 ml., is placed in the oil so as to rest in the dimple of the specimen, then the beaker is stored at  $140^{\circ} \pm 2^{\circ}$  F. and observed daily for failure of the specimen, i. e., the first sign of rust which increases in intensity the following day. Four test specimens are run. Where the water drop slowly disappears, it is restored by addition thereto to original size when it reaches 50% of its original diameter. Three of the four specimens should be free of rust for the test period in order to pass test.

In summation, it has been found that, contrary to expectations, when about 0.1 percent by weight of the basic nitrogen-containing polymerization-inhibiting and corrosion-inhibiting additives of our composition are added to a lubricant incorporating a fatty ester or a mixture of fatty esters which have been phosphorized and/or phosphorized-sulfurized, the promotion of polymerization of said fatty ester, or esters thought to be brought about by the presence of phosphorus, particularly phosphorus in the presence of sulfur, is counteracted so that satisfactory stability of the lubricant is achieved. Furthermore, extreme pressure lubricants containing the above-mentioned constituents incorporated in a mineral oil fraction exhibit corrosion inhibition. The polymerization-inhibiting and the corrosion-inhibiting characteristics of the formulation are present both during storage of the lubricant and during use of the lubricant under conditions of extreme pressure and elevated temperatures.

The constituents of our composition may be added together in any suitable manner, that is, with or without stirring, in conventional apparatus, and any sequence; the constituents may be added intermittently, continuously, swiftly or slowly, in any order to achieve a homogeneous extreme pressure lubricant.

In addition, the composition of our invention which comprises a petroleum base oil, together with the extreme pressure and the polymerization-inhibiting and corrosion-inhibiting additives indicated, may include other conventional lubricating oil additives added to the composition for known specific properties, and which do not substantially interfere with extreme pressure characteristics, polymerization-inhibition, or corrosion-inhibition. Such additional additives may be viscosity index improvers, such as, "Paratone" a polyisobutylene polymer, "Acryloid" polymers of the esters of methacrylic acid and higher fatty alcohol, and "Santodex," an alkyl styrene polymer;

"Paraflo" a complex condensation product of paraffin wax and naphthalene, "Santopour," a paraffin wax, phenolic condensation product, and "Acryloid" described above; and other assisting agents, for example, foam depressants such as Dow Corning Fluid DC-200, a silicone polymer, and Monsanto Chemical Company's PC-1308, and the like.

Whenever the terms "Armeen-S," "Armeen-HTD," "Duomeen-T" and "Duomeen-T Dioleate" are used in 10 the claims they shall mean the substance as defined in the foregoing specification.

We claim:

1. An extreme pressure lubricant which comprises a mineral oil, an amount sufficient to impart extreme pressure properties to the oil of extreme pressure additive comprising a phosphorized and sulfurized ester of a fatty acid and aliphatic alcohol, and a nitrogen-containing compound comprising at least one member of the group consisting of aliphatic amines having at least one carbon chain of at least 16 carbon atoms, aliphatic amides having at least one carbon chain of at least 16 carbon atoms and aliphatic amine salts of fatty acids of carbon chain of at least 16 carbon atoms, wherein the amine radical has at least 16 carbon atoms, in a polymerization-inhibiting amount.
2. An extreme pressure lubricant which comprises a major amount of a petroleum lubricating oil, an amount sufficient to impart extreme pressure properties to said oil of a phosphorized and sulfurized ester of a fatty acid 30 of carbon chain length of at least 12 carbon atoms and a lower aliphatic alcohol, and a nitrogen-containing compound comprising at least one member of the group consisting of fatty amines having at least one carbon chain of at least 16 carbon atoms and not more than 22 carbon atoms, fatty amides having at least one carbon chain of at least 16 carbon atoms and not more than 22 carbon atoms, and aliphatic amine salts of fatty acids of carbon chain length of at least 16 carbon atoms and not more than 22 carbon atoms, wherein the amine radical has at 40 least 16 carbon atoms and not more than 22 carbon atoms, in a polymerization-inhibiting amount.
3. An extreme pressure lubricant which comprises a major amount of a petroleum lubricating oil, an amount sufficient to impart extreme pressure properties to the 45 said lubricating oil of a mixture of esters, which have been phosphorized and sulfurized with phosphorus sesquisulfide, of fatty acids of carbon chain lengths of at least 12 carbon atoms and lower aliphatic alcohols, and a nitrogen-containing compound comprising at least one 50 member of the group consisting of fatty amines of carbon chain lengths of at least 16 carbon atoms and not more than 22 carbon atoms, fatty amides of carbon chain length of at least 16 carbon atoms and not more than 22 carbon atoms, and aliphatic amine salts of fatty acids of 55 carbon chain length of at least 16 carbon atoms and not more than 22 carbon atoms wherein the amine radical has at least 16 carbon atoms and not more than 18 carbon atoms, in a polymerization-inhibiting amount.
4. An extreme pressure lubricant which comprises a 60 major amount of a petroleum lubricating oil, a sulfurized ester, of tall oil and a lower aliphatic alcohol, in combination with an ester of a fatty acid of carbon chain length of at least 16 carbon atoms and a trihydroxy alcohol, which ester has been chemically reacted with phosphorus sesquisulfide, the latter two components in an amount sufficient to impart extreme pressure properties to the oil, and at least about 0.1 percent by weight of the total composition, sufficient to inhibit polymerization, of a nitrogen-containing compound comprising at least one member of the group consisting of fatty amines having at least one carbon chain of at least 16 carbon atoms and not more than 22 carbon atoms, fatty amides having at least one carbon chain of at least 16 carbon atoms and not more than 22 carbon atoms, and aliphatic amine salts of fatty acids of at least 65 16 carbon atoms and

not more than 22 carbon atoms wherein the amine radical has an alkyl substituent which has at least 18 carbon atoms and not more than 19 carbon atoms.

5. An extreme pressure lubricant which comprises a mineral oil in major amount, an amount sufficient to impart extreme pressure qualities to said mineral oil of at least one phosphorus-containing ester of a fatty acid of carbon chain length of at least 12 carbon atoms and a lower aliphatic alcohol, obtained by reacting said ester with a phosphorus sulfide and an aliphatic amine having at least one carbon chain of at least 16 carbon atoms and not more than 22 carbon atoms in an amount sufficient to inhibit sediment formation in the composition.

6. The lubricant of claim 5 in which said amine has at least one hydrogen atom attached to at least one nitrogen atom.

7. An extreme pressure lubricant which comprises a mineral oil in a major amount, an amount sufficient to impart extreme pressure qualities to said mineral oil of at least one phosphorus-containing ester of a fatty acid of carbon chain length of at least 12 carbon atoms and a lower aliphatic alcohol, obtained by reacting said ester with a phosphorus sulfide and an aliphatic amide having at least one carbon chain of at least 16 carbon atoms and not more than 22 carbon atoms in an amount sufficient to inhibit sediment formation in the composition.

8. An extreme pressure lubricant which comprises a petroleum lubricating oil in a major amount, an amount sufficient to impart extreme pressure qualities to said petroleum lubricating oil of at least one phosphorus-containing ester of a fatty acid of carbon chain length of at least 12 carbon atoms and a lower aliphatic alcohol, obtained by reacting said ester with a phosphorus sulfide and an aliphatic amine salt of a fatty acid of carbon chain length of at least 16 carbon atoms and not more than 22 carbon atoms, wherein said amine radical has at least 16 carbon atoms and not more than 22 carbon atoms, in an amount sufficient to inhibit sediment formation in the composition.

9. The lubricant of claim 8 in which said aliphatic amine salt is an alkyl substituted trimethylene diamine salt.

10. An extreme pressure lubricant which comprises a petroleum lubricating oil in major amount, an amount sufficient to impart extreme pressure qualities to said petroleum lubricating oil of at least one sulfurized and phosphorized ester of a fatty acid of carbon chain length of at least 12 carbon atoms and a lower aliphatic alcohol, and an aliphatic amine having at least one carbon chain of at least 16 carbon atom and not more than 22 carbon atoms in an amount sufficient to inhibit sediment formation in the composition.

11. The lubricant of claim 10 in which said amine has at least one hydrogen atom attached to at least one nitrogen atom.

12. An extreme pressure lubricant which comprises a petroleum lubricating oil in a major amount, an amount sufficient to impart extreme pressure qualities to said hydrocarbon petroleum lubricating oil of at least one sulfurized and phosphorized ester of a fatty acid of carbon chain length of at least 12 carbon atoms and a lower aliphatic alcohol, and an aliphatic amide having at least one carbon chain of at least 16 carbon atoms and not more than 22 carbon atoms in an amount sufficient to inhibit sediment formation in the composition.

13. An extreme pressure lubricant which comprises a petroleum lubricating oil in a major amount, an amount sufficient to impart extreme pressure qualities to said petroleum lubricating oil of at least one sulfurized and phosphorized ester of a fatty acid of carbon chain length of at least 12 carbon atoms and a lower aliphatic alcohol, and an aliphatic amine salt of a fatty acid of carbon chain length of at least 16 carbon atoms and not more than 22 carbon atoms, wherein said amine radical has at least 16 carbon atoms and not more than 22 carbon

atoms, in an amount sufficient to inhibit sediment formation in the composition.

14. The lubricant of claim 13 in which the amine salt is an alkyl substituted trimethylene diamine salt.

5 15. An extreme pressure lubricant which comprises a major amount of petroleum lubricating oil, a minor extreme pressure-imparting amount of an extreme pressure additive which comprises sulfurized methyl esters of tall oil and glycerol trioleate phosphorized-sulfurized with phosphorus sesquisulfide, in a ratio of one to ten parts tall oil esters to one part glycerol trioleate, and a minor amount of a mixture of fatty amines containing 10 parts of hexadecylamine, 10 parts of octadecylamine, 35 parts of octadecenylamine and 45 parts of octadecyldienylamine, sufficient to inhibit polymer formation.

10 16. An extreme pressure lubricant which comprises about 56 percent by weight of 150 viscosity bright stock oil, about 31.9 percent by weight of 170 viscosity neutral oil, about 10 percent by weight of an extreme pressure additive which comprises sulfurized methyl esters of tall oil and glycerol trioleate phosphorized-sulfurized with phosphorus sesquisulfide, in a ratio of one to ten parts tall oil esters to one part glycerol trioleate, about 1 percent by weight of dibenzyl disulfide, about 1 percent by weight, as a viscosity index improver, of the polymer of mixed cetyl, octyl and lauryl esters of methacrylic acid having 10,000-20,000 molecular weight and about 0.1 percent by weight of a mixture of fatty amines containing 10 parts of hexadecylamine, 10 parts of octadecylamine, 35 parts of octadecenylamine and 45 parts of octadecyldienylamine.

15 17. An extreme pressure lubricant which comprises a major amount of a petroleum lubricating oil, a minor extreme pressure-imparting amount of an extreme pressure additive which comprises sulfurized methyl esters of tall oil and glycerol trioleate phosphorized-sulfurized with phosphorus sesquisulfide, in a ratio of one to ten parts tall oil esters to one part glycerol trioleate, and a minor amount of a compound having the formula



20 sufficient to inhibit polymer formation.

25 18. An extreme pressure lubricant which comprises about 56 percent by weight of 150 viscosity bright stock oil, about 31.9 percent by weight of 170 viscosity neutral oil, about 0.1 percent by weight of a compound having the formula



30 25 19. An extreme pressure lubricant which comprises about 1 percent by weight of dibenzyl disulfide, about 1 percent by weight, as a viscosity index improver, of the polymer of mixed cetyl, octyl and lauryl esters of methacrylic acid having 10,000-20,000 molecular weight, and about 10 percent by weight of an extreme pressure additive which comprises 3 parts of sulfurized methyl esters of tall oil and one part of glycerol trioleate which has been phosphorized-sulfurized with phosphorus sesquisulfide.

35 20. An extreme pressure lubricant which comprises a major amount of a petroleum lubricating oil, a minor extreme pressure-imparting amount of an extreme pressure additive which comprises sulfurized methyl esters of tall oil and glycerol trioleate phosphorized-sulfurized with phosphorus sesquisulfide, in a ratio of one to ten parts tall oil esters to one part glycerol trioleate, and a minor amount of stearylamide sufficient to inhibit polymer formation.

40 75 21. An extreme pressure lubricant which comprises about 56 percent by weight of 150 viscosity bright stock oil, about 31.9 percent by weight of 170 viscosity neutral

oil, about 0.1 percent by weight of stearyl amide, about 1 percent by weight of dibenzyl disulfide, about 1 percent by weight, as a viscosity index improver, of the polymer of mixed cetyl, octyl and lauryl esters of methacrylic acid having 10,000-20,000 molecular weight, and about 10 percent by weight of an extreme pressure additive comprising 3 parts of sulfurized methyl esters of tall oil and one part of glycerol trioleate which has been phosphorized-sulfurized by phosphorus sesquisulfide.

5

## References Cited in the file of this patent

## UNITED STATES PATENTS

|           |         |       |               |
|-----------|---------|-------|---------------|
| 2,151,300 | Moran   | ----- | Mar. 21, 1939 |
| 2,268,608 | McNulty | ----- | Jan. 6, 1947  |